# EUROPEAN PATENT APPLICATION

(11) **EP 4 778 652 A1**
(43) Date of publication of application: **22.07.2026**
(21) Application number: 24937935.5
(22) Date of filing: 20.11.2024
(51) Int. Cl.: B22F 1/16, B22F 1/00, B22F 1/05, B22F 1/10, B22F 1/054, B22F 1/102, B22F 3/24, B22F 3/105

(54) **CARBON-COATED METAL POWDER AND PASTE**

(30) Priority: 30.04.2024 JP 2024074071
(71) Applicant: JX Advanced Metals Corporation, Tokyo 105-8417 (JP)
(72) Inventor: TSUCHIDA,Katsuyuki, Kitaibaraki-shi, Ibaraki 319-1535 (JP); ISE,Naoki, Kitaibaraki-shi, Ibaraki 319-1535 (JP); GOTO,Yuki, Kitaibaraki-shi, Ibaraki 319-1535 (JP)
(74) Representative: Yeadon IP Limited
(86) International application number: PCT/JP2024/041178
(87) International publication number: WO 2025/229771

(57) **Abstract**

A carbon-coated metal powder comprising metal particles and a coating layer covering at least a portion of a surface of the metal particles, the coating layer containing carbon, wherein the metal particles consist of (1) tin, copper, or silver and inevitable impurities, or (2) an alloy of tin, copper, or silver having a tin, copper, or silver content of 50 mass% or more, respectively, and inevitable impurities, and wherein a mean particle diameter calculated from BET specific surface area is 150 nm or less.

## Description

### FIELD OF THE INVENTION

The present specification describes a carbon-coated metal powder and a paste.

### BACKGROUND OF THE INVENTION

Metal powder composed of a predetermined pure metal or alloy may be mixed with a liquid containing organic matter such as an organic binder or an organic solvent to form a paste. Such pastes may be used, for example, as pastes for electronic device materials or energy device materials typified by conductive pastes for forming wiring by printing, filling holes, or bonding, or as solder pastes used for soldering.

Although not related to metal powders for pastes, Patent Document 1, for example, proposes a carbon-coated metal powder under the object of "providing a carbon-coated metal powder and the like that is excellent in fluidity, capable of efficient absorption of energy beams, and suitable for use as a powder material for additive manufacturing," wherein the proposed powder is "a carbon-coated metal powder having a carbon coating formed by chemically coating the surface of metal particles having an average particle diameter of 1 µm or more and 100 µm or less with carbon derived from an organic compound, wherein the amount of the carbon coating in the carbon-coated metal powder is 0.001 mass% or more and 2.0 mass% or less."

### CITATION LIST

### Patent Literatures

[Patent Literature 1] Japanese Unexamined Patent Publication No. 2018-199862

### SUMMARY OF THE INVENTION

Depending on the application, metal powder may be required to have a smaller particle diameter than the "average particle diameter of 1 µm or more and 100 µm or less" described in Patent Document 1. Reducing the particle diameter of the metal powder offers advantages such as, for example, a lower melting point due to increased surface area and higher activity, thereby lowering the melting temperature, and the ability to apply the powder as a thin film or to narrow areas when formed into a paste.

However, such extremely fine metal powder has a larger surface area, which makes it more susceptible to oxidation. Upon oxidation, the proportion of metal in the total metal particles decreases. For example, when fine metal powder of Cu or Ag is formed into a paste and used as a wiring material, a problem arises in that electrical conductivity decreases due to oxidation. In the case of fine metal powder of Sn, oxidation of the surface reduces the melting of Sn, and the function as a solder paste deteriorates. In addition, extremely fine metal powder tends to aggregate among metal particles when left as is or when mixed with a liquid such as a paste. For example, a paste containing aggregated metal powder may result in non-uniform application due to the presence of such aggregates when applied as a thin film or to a narrow area, potentially causing defects attributable thereto.

In view of such problems, embodiments of the present invention provide a carbon-coated metal powder having a relatively small particle diameter and capable of effectively suppressing surface oxidation and aggregation in powder form or in a liquid such as a paste, as well as a paste comprising the same.

Embodiments of the present invention that solve the above problem are defined below.
[1] A carbon-coated metal powder comprising:
   metal particles; and
   a coating layer covering at least a portion of a surface of the metal particles, the coating layer containing carbon,
   wherein the metal particles comprise (1) tin, copper, or silver and inevitable impurities, or (2) an alloy of tin, copper, or silver having a tin, copper, or silver content of 50 mass% or more, respectively, and inevitable impurities, and
   wherein a mean particle diameter calculated from BET specific surface area is 150 nm or less.
[2] The carbon-coated metal powder according to [1], wherein the carbon content is 0.5 to 3.0 mass%.
[3] The carbon-coated metal powder according to [1] or [2], wherein the hydrogen content is 0.01 to 0.25 mass%.
[4] The carbon-coated metal powder according to any one of [1] to [3], wherein the coating layer containing carbon is composed of a mixture of graphitic carbon and a hydrocarbon.
[5] The carbon-coated metal powder according to any one of [1] to [4], wherein the oxygen content is 3.0 mass% or less.
[6] The carbon-coated metal powder according to any one of [1] to [5], which is used in a paste.
[7] A paste comprising the carbon-coated metal powder according to any one of [1] to [6], and a liquid containing organic matter.

According to embodiments of the present invention, it is possible to provide a carbon-coated metal powder having a relatively small particle diameter and capable of effectively suppressing surface oxidation and aggregation in powder form or in a liquid such as a paste, as well as a paste comprising the same.

### BRIEF DESCRIPTION OF THE DRAWINGS

FIG. 1 is a cross-sectional view schematically illustrating surface-coated particles contained in the carbon-coated metal powder according to an embodiment of the present invention.
FIG. 2 is SEM images of the carbon-coated metal powders according to Examples 1 to 3.
FIG. 3 is SEM images of the metal powder according to Comparative Example 1.
FIG. 4 is SEM images of coarse particles in the carbon-coated metal powder according to Example 1.
FIG. 5 is SEM images of coarse particles in the metal powder according to Comparative Example 1.
FIG. 6 is a Raman spectrum of the carbon-coated metal powder according to Example 3.
FIG. 7 is a Raman spectrum of the metal powder according to Comparative Example 1.
FIG. 8 shows photographs showing the appearance when the carbon-coated metal powder according to Example 1 is mixed with silicone oil.
FIG. 9 shows photographs showing the appearance when the carbon-coated metal powder according to Example 1 is mixed with PEG 1000.
FIG. 10 shows photographs showing the appearance when the carbon-coated metal powder according to Example 1 is mixed with carbon paste.

### DETAILED DESCRIPTION OF THE INVENTION

Hereinafter, preferred embodiments of the present invention will be described in detail; however, the present invention should not be construed as being limited thereto. Various modifications and improvements may be made based on the knowledge of those skilled in the art without departing from the gist of the present invention. A plurality of constituent elements disclosed in the embodiments may be combined appropriately to form various inventions. For example, some constituent elements may be omitted from all of the constituent elements shown in the embodiments.

### <Carbon-Coated Metal Powder>

The carbon-coated metal powder according to an embodiment of the present invention comprises metal particles and a coating layer covering at least a portion of a surface of the metal particles, the coating layer containing carbon, wherein the metal particles consist of (1) tin, copper, or silver and inevitable impurities, or (2) an alloy of tin, copper, or silver having a tin, copper, or silver content of 50 mass% or more, respectively, and inevitable impurities, and wherein a mean particle diameter calculated from BET specific surface area is 150 nm or less.

More specifically, the carbon-coated metal powder according to an embodiment of the present invention is an aggregate of particles comprising surface-coated particles 3 in which metal particles 1 are covered with a coating layer 2, as illustrated in FIG. 1, and most or substantially all of the aggregate is composed of surface-coated particles 3. In surface-coated particle 3 shown in FIG. 1, the entire surface of metal particle 1 is covered with coating layer 2; however, it is sufficient that coating layer 2 is adhered to the surface of metal particle 1 so as to cover at least a portion of the surface of metal particle 1. In other words, a portion of the surface of metal particle 1 may remain exposed without being covered by coating layer 2.

As described above, the carbon-coated metal powder according to an embodiment of the present invention has a relatively small mean particle diameter of 150 nm or less, while exhibiting excellent dispersibility in liquids such as pastes. Although the reason is not entirely clear, it is believed that the compatibility with the paste is improved because at least a portion of the surface of the metal particles is covered with the coating layer containing carbon. The mean particle diameter of the carbon-coated metal powder according to an embodiment of the present invention may be 120 nm or less, or may be 100 nm or less. The coating layer containing carbon also functions to suppress oxidation of the surface of the metal particles. The mean particle diameter of the carbon-coated metal powder according to an embodiment of the present invention can be measured using a Macsorb/HM model-1208 manufactured by MOUNTEC Co., Ltd.

### (Composition)

The metal particles contained in the carbon-coated metal powder according to an embodiment of the present invention consist of (1) tin, copper, or silver and inevitable impurities. Alternatively, the metal particles contained in the carbon-coated metal powder according to an embodiment of the present invention consist of (2) an alloy of tin, copper, or silver having a tin, copper, or silver content of 50 mass% or more, respectively, and inevitable impurities.

When the metal particles of the carbon-coated metal powder according to an embodiment of the present invention contain a metal, the tin, copper, or silver content in the metal portion of the carbon-coated metal powder may be, for example, 99.0 mass% or more, typically 99.9 mass% or more, and preferably 99.99 mass% or more.

When the metal particles of the carbon-coated metal powder according to an embodiment of the present invention contain an alloy, the tin, copper, or silver content in the carbon-coated metal powder is 50 mass% or more, respectively. The tin, copper, or silver content in the carbon-coated metal powder is more preferably 60 mass% or more, respectively. For such alloys of tin, copper, or silver, the tin, copper, or silver content in the carbon-coated metal powder is preferably controlled according to the application and other factors. For example, in carbon-coated metal powder used in solder paste, specific examples of alloys constituting the metal particles include alloys having compositions of 63%Sn-37%Pb, 60%Sn-40%Pb, 96.5%Sn-3%Ag-0.5%Cu, 95%Sn-4%Ag-1%Cu, and 95%Sn-5%Ag in mass% ratio.

Inevitable impurities contained in the metal particles of the carbon-coated metal powder according to an embodiment of the present invention include Si, Fe, Na, Mg, and the like. The content of inevitable impurities contained in the metal particles of the carbon-coated metal powder is preferably 1.0 mass% or less, and more preferably 0.1 mass% or less. It should be noted that when multiple types of inevitable impurities are present, the content of inevitable impurities refers to the total content thereof.

The tin, copper, or silver content in the carbon-coated metal powder, as well as the content of additive elements and the content of impurities when the metal particles are an alloy, can be measured by ICP-MS when the sample to be measured is in liquid form, or by GD-MS when in solid form. For example, the carbon-coated metal powder as a solid sample may be placed in a measurement container, compacted by applying pressure, and then measured by GD-MS. The impurity content can be analyzed, for example, as a ratio (ppm) relative to Sn.

Since the carbon-coated metal powder according to an embodiment of the present invention contains a coating layer containing carbon, it contains carbon. The carbon content of the carbon-coated metal powder is preferably 0.5 to 3.0 mass%, and more preferably 0.5 to 2.0 mass%. If the carbon content is too low, there is a concern that suppression of aggregation and oxidation will be insufficient. On the other hand, if the carbon content is too high, electrical conductivity between particles may decrease, or the surface may become inert, which could inhibit fusion between particles upon heating. The carbon-coated metal powder according to an embodiment of the present invention may be configured such that the coating layer containing carbon is composed of a mixture of graphitic carbon and a hydrocarbon. Here, graphitic carbon is generated by heating a hydrocarbon in an inert atmosphere (e.g., a gas atmosphere such as nitrogen or argon) or in a sealed air environment, and the coating of metal powder can be formed by spraying a hydrocarbon such as methane onto heated metal powder. Graphitic carbon is detected by Raman analysis as a "D band" peak near Raman shift 1350 cm⁻¹, a "G band" peak near 1600 cm⁻¹, and a 2D band or G' band peak near 2680 cm⁻¹. As such, it is preferable that the coating layer of the carbon-coated metal powder contains a hydrocarbon, and the hydrogen content is preferably 0.01 to 0.25 mass%, and more preferably 0.01 to 0.1 mass%. As the hydrogen content increases, compatibility with the paste improves, leading to better dispersibility. Since the hydrogen contained in this coating layer is hydrogen from hydrocarbons such as methane, if the hydrogen content is too high, the carbon content also increases, which may decrease electrical conductivity between particles or cause the surface to become inert, inhibiting fusion between particles upon heating. The carbon content or hydrogen content of the carbon-coated metal powder can be analyzed by non-dispersive infrared absorption spectrometry and measured as a ratio (ppm) relative to the total mass of the carbon-coated metal powder.

In the carbon-coated metal powder according to an embodiment of the present invention, the metal particles are covered with the coating layer containing carbon, thereby suppressing oxidation of the metal particles and resulting in a powder that contains substantially no oxygen or has a low oxygen content. The oxygen content of the carbon-coated metal powder may be, for example, 3.0 mass% or less, typically 2.5 mass% or less, or further 1.5 mass% or less. A low oxygen content is believed to facilitate melting of the metal upon heating. The oxygen content can be analyzed by non-dispersive infrared absorption spectrometry and measured as a ratio (ppm) relative to the total mass of the carbon-coated metal powder.

### (Particle Diameter)

The carbon-coated metal powder according to an embodiment of the present invention has a relatively small particle diameter. Specifically, the mean particle diameter calculated from BET specific surface area (referred to as the BET diameter) of the carbon-coated metal powder is 150 nm or less, typically 100 nm or less, and may more typically be 50 to 80 nm. If the mean particle diameter is too large, it becomes difficult to form a thin film when applied as a paste. Increasing the mean particle diameter may improve handleability and may allow for less susceptibility to aggregation.

The BET specific surface area of the carbon-coated metal powder according to an embodiment of the present invention can be measured in accordance with JIS Z 8830:2013 using, for example, a Macsorb/HM model-1208 manufactured by MOUNTEC Co., Ltd. The mean particle diameter d (µm) calculated from BET specific surface area can be calculated from the BET specific surface area using the formula: d = 6/(ρ × s). In this formula, ρ is the density (g/cm³) of tin, copper, or silver, or the density (g/cm³) of an alloy of tin, copper, or silver, as determined according to the composition of the metal particles, and s is the BET specific surface area (m²/g).

When acquiring SEM images at 2,000× magnification of the carbon-coated metal powder according to an embodiment of the present invention, observations are carried out over as wide a range as possible to confirm the presence or absence of coarse particles. For example, it is sufficient to observe 10 to 20 fields of view of the SEM image at 2,000× magnification. At this time, it is preferable that there are 2 or fewer coarse particles with a particle diameter of 5 µm or more, more preferably 1 or fewer, and most preferably 0. Such a configuration makes it even easier to achieve thin film application or highly accurate printing in narrow areas during paste application. The "particle diameter" referred to herein can be measured by scanning electron microscopy (SEM).

### (Production Method)

As a method for producing the carbon-coated metal powder according to an embodiment of the present invention, it is preferable to first prepare a large metal powder having a particle diameter of several µm to several tens of µm produced by gas atomization or the like, and then to refine the metal powder by RF plasma. In RF plasma, the metal on the surface of the metal particles of the metal powder evaporates, reducing the diameter of the metal particles.

Then, while the metal powder is in a high-temperature state following RF plasma processing, a hydrocarbon-based gas containing methane or the like can be sprayed onto the metal powder. At this time, decomposition and carbonization reactions occur on the surface of the metal particles due to the spraying of the hydrocarbon-based gas, and a coating layer containing carbon is formed thereon. At this stage, the proportion of hydrocarbon in the carbon coating can be varied by changing the amount of gas sprayed. If necessary, air classification or other classification may be performed after the RF plasma processing to remove coarse particles.

In this manner, a carbon-coated metal powder is obtained having a predetermined small mean particle diameter and comprising surface-coated particles in which at least a portion of the surface of the metal particles is covered with a coating layer. In such a carbon-coated metal powder, since at least a portion of the surface of the metal particles is covered with the coating layer, the metal particles are resistant to oxidation and the oxygen content is relatively low.

### <Paste>

The carbon-coated metal powder according to an embodiment of the present invention described above is preferably used in a conductive paste, a solder paste, or other pastes. Such a paste contains a liquid containing organic matter in addition to the carbon-coated metal powder according to an embodiment of the present invention, and may be produced by, for example, mixing and stirring the carbon-coated metal powder according to an embodiment of the present invention with a liquid containing organic matter.

The liquid containing organic matter in the paste may include an organic binder, an organic solvent, and the like. Commonly used materials may be used as the organic binder and organic solvent.

### EXAMPLES

The carbon-coated metal powder described above was produced on a trial basis and its effects were confirmed, as described below. However, this description is for illustrative purposes only and is not intended to be limiting.

For Examples 1 to 3, atomized powder (mean particle diameter D50: 5.5 µm) manufactured by Nippon Atomized Metal Powders Corporation was prepared as a raw material.

For each of the raw materials of Examples 1 to 3, the powder was refined by RF plasma at different output levels, and after RF plasma processing, methane was sprayed to apply a carbon coating. In all of Examples 1 to 3, the conditions for RF plasma and methane spraying were kept the same.

In this manner, samples of the carbon-coated metal powder according to Examples 1 to 3 were produced.

For Comparative Example 1, Sn powder (purity 99.7%) manufactured by Kanto Chemical Co., Inc. was prepared as a raw material, and this was used as the metal powder sample according to Comparative Example 1.

### (BET Diameter)

The BET diameter (mean particle diameter calculated from BET specific surface area) of the samples of carbon-coated metal powder according to Examples 1 to 3 and metal powder according to Comparative Example 1 was measured as follows.

The BET specific surface area was measured by the BET method in accordance with JIS Z 8830:2013 using a Macsorb/HM model-1208 manufactured by MOUNTEC Co., Ltd. The mean particle diameter d calculated from BET specific surface area was calculated from the BET specific surface area using the formula: d = 6/(ρ × s). In this formula, ρ is the density (g/cm³) of tin, copper, or silver, or the density (g/cm³) of an alloy of tin, copper, or silver, as determined according to the composition of the metal particles, and s is the BET specific surface area (m²/g).

The obtained BET diameters (mean particle diameters calculated from BET specific surface area) are shown in Table 1.

**Table 1**

| | BET diameter (nm) |
|---|---|
| EX. 1 | 92.1 |
| EX. 2 | 63.6 |
| EX. 3 | 102.1 |
| Comp. EX. 1 | 117.7 |

### (XRD Measurement)

The samples of the carbon-coated metal powder according to Examples 1 to 3 were measured using the following XRD diffractometer. Based on the obtained XRD spectra of Examples 1 to 3, it was found that the samples of the carbon-coated metal powder according to Examples 1 to 3 were pure tin.

### (SEM Observation)

The samples of the carbon-coated metal powder according to Examples 1 to 3 and the metal powder according to Comparative Example 1 were observed using a scanning electron microscope (SEM): JXA-8500F (5CH) manufactured by JEOL Ltd. at an acceleration voltage of 15.0 kV and magnifications of 2,000× and 10,000×. The obtained SEM images are shown in FIGS. 2 to 3. As shown in FIG. 2, it was confirmed that the carbon-coated metal powders according to Examples 1 to 3 were all particles of several tens of nm. As shown in FIG. 3, it was confirmed that the metal powder according to Comparative Example 1 was aggregated.

In addition, for the samples of the carbon-coated metal powder according to Examples 1 to 3 and the metal powder according to Comparative Example 1, SEM observation (magnification: 2,000×) was conducted at 20 locations in the same manner as described above to search for coarse particles.

As a result, in Example 1, relatively many coarse particles with a particle diameter of 1 to 2 µm were observed, but no coarse particles with a particle diameter of 5 µm or more were found. SEM images of the coarse particles with a particle diameter of 1 to 2 µm in Example 1 are shown in FIG. 4.

In Examples 2 and 3 as well, no coarse particles with a particle diameter of 5 µm or more were found.

In Comparative Example 1, coarse particles with a particle diameter of approximately 30 µm were found, as shown in FIG. 5.

### (Structural Analysis of Coating Layer Containing Carbon)

The samples of the carbon-coated metal powder according to Example 3 and the metal powder according to Comparative Example 1 were measured using a micro-Raman spectrometer manufactured by Renishaw plc at a laser wavelength of 532 nm over a Raman shift range of 100 to 3500 cm⁻¹ with 100 accumulations, and structural analysis was performed using Raman spectra. The Raman spectrum of the carbon-coated metal powder according to Example 3 is shown in FIG. 6, and the Raman spectrum of the metal powder according to Comparative Example 1 is shown in FIG. 7.

For Example 3, a "D band" peak near Raman shift 1350 cm⁻¹, a "G band" peak near 1600 cm⁻¹, and a 2D band or G' band peak near 2680 cm⁻¹ were detected, confirming the presence of graphitic carbon. In addition, peaks attributable to CH bonds were obtained at 2931 cm⁻¹ and 3221 cm⁻¹, confirming the presence of hydrocarbon. Thus, it was found that the carbon-coated metal powder according to Example 3 is a mixture of graphitic carbon and hydrocarbon.

For Comparative Example 1, as shown in FIG. 7, no peaks derived from graphitic carbon or hydrocarbon were detected.

For the samples of the carbon-coated metal powder according to Examples 1 to 3 and the metal powder according to Comparative Example 1, the contents of carbon (C), hydrogen (H), nitrogen (N), oxygen (O), and sulfur (S) were analyzed by non-dispersive infrared absorption spectrometry (LECO Japan G.K., model numbers: CS600 (C, S), TC600 (O, N), TCH600 (H)), and measured as ratios (ppm) relative to the total mass of the carbon-coated metal powder. Similarly, the total content of impurities excluding C, H, N, O, and S was analyzed and measured as a ratio (ppm) relative to the total mass of the carbon-coated metal powder. The measurement results are shown in Table 2.

As shown in Table 2, for Examples 1 to 3, the carbon content was 0.5 to 3.0 mass% (5,000 to 30,000 ppm), the hydrogen content was 0.01 to 0.25 mass% (100 to 2,500 ppm), and the oxygen content was 3.0 mass% or less (30,000 ppm or less). On the other hand, for Comparative Example 1, the oxygen content was extremely high at 8 mass% (80,000 ppm). The hydrogen content was also high; however, based on the results of the Raman spectra described above, it is believed that this was not due to hydrocarbon but rather to hydrogen from hydroxyl groups.

**Table 2**

| | EX.1 | EX.2 | EX.3 | Comp. EX.1 |
|---|---|---|---|---|
| | (ppm) | (ppm) | (ppm) | (ppm) |
| C | 8000 | 27000 | 17000 | 420 |
| N | 20 | <10 | <10 | <10 |
| O | 11000 | 8600 | 5900 | 80000 |
| S | <10 | <10 | <10 | 30 |
| H | 390 | 320 | 220 | 1600 |
| impurities | 107 | 85 | 44 | 1056 |

### (Dispersibility)

To confirm dispersibility, 0.05 g of the carbon-coated metal powder sample according to Example 1 was added to 5.00 g of various viscous liquids (silicone oil, polyethylene glycol (PEG 1000), or carbon paste) and mixed with a pencil mixer. Note that for polyethylene glycol (PEG 1000), the carbon-coated metal powder was added and mixed after the liquid was heated to 50°C to liquefy it. Photographs thereof are shown in FIGS. 8 to 10.

As can be seen from FIGS. 8 to 10, it was confirmed that the carbon-coated metal powder could be uniformly mixed in all cases, as observed visually. This suggested that the aforementioned carbon-coated metal powder, although having a relatively small particle diameter, has the potential to effectively suppress aggregation in liquids.

### (Melting Point and Endothermic Amount)

To confirm the melting point and endothermic amount of the samples of the carbon-coated metal powder according to Examples 1 to 3 and the metal powder according to Comparative Example 1, differential scanning calorimetry (DSC) was performed. The DSC apparatus used was a Thermo plus EVOS series DSC8231 manufactured by Rigaku Corporation, and measurements were taken under the following conditions. The evaluation results are shown in Table 3.
- Measurement atmosphere: N₂, heating rate: 5°C/min, measurement temperature: room temperature to 300°C

| | Endothermic peak starting point (°C) | Endothermic amount (J/g) |
|---|---|---|
| Comp. EX.1 | 219 | 32.562 |
| EX.1 | 216 | 36.509 |
| EX.2 | 220 | 37.437 |
| EX.3 | 221 | 41.761 |

From Table 3, it was confirmed that Examples 1 to 3, which are carbon-coated metal powders, had larger endothermic amounts than Comparative Example 1, which is a metal powder without carbon coating, due to suppressed oxidation. In addition, while the melting point of bulk Sn is 232°C, the melting points (endothermic peak onset temperatures) of the carbon-coated metal powders according to Examples 1 to 3 were 216 to 221°C, which are lower than that of bulk Sn, confirming that they have higher activity.

### (Potential Contribution to SDGs)

According to the embodiments described above, since aggregation in liquids can be effectively suppressed, there is a possibility that the yield and performance of products manufactured using carbon-coated metal powder can be improved. For this reason, these embodiments may potentially contribute to Goal 9 "Build resilient infrastructure, promote inclusive and sustainable industrialization, and foster innovation" and Goal 12 "Ensure sustainable consumption and production patterns" of the Sustainable Development Goals (SDGs) led by the United Nations.

### Description of Reference Numerals

1: Metal particle
2: Coating layer
3: Surface-coated particle

## Claims

1. A carbon-coated metal powder comprising:
metal particles; and
a coating layer covering at least a portion of a surface of the metal particles, the coating layer containing carbon,
wherein the metal particles comprise (1) tin, copper, or silver and inevitable impurities, or (2) an alloy of tin, copper, or silver having a tin, copper, or silver content of 50 mass% or more, respectively, and inevitable impurities, and
wherein a mean particle diameter calculated from BET specific surface area is 150 nm or less.

2. The carbon-coated metal powder according to claim 1, wherein the carbon content is 0.5 to 3.0 mass%.

3. The carbon-coated metal powder according to claim 1, wherein the hydrogen content is 0.01 to 0.25 mass%.

4. The carbon-coated metal powder according to claim 1, wherein the coating layer containing carbon is composed of a mixture of graphitic carbon and a hydrocarbon.

5. The carbon-coated metal powder according to claim 1, wherein the oxygen content is 3.0 mass% or less.

6. The carbon-coated metal powder according to claim 1, which is used in a paste.

7. A paste comprising the carbon-coated metal powder according to any one of claims 1 to 6, and a liquid containing organic matter.
